

## UNITED STATES PATENT OFFICE.

MORITZ JOSEPH HEITMANN, OF FREITAL-POTSCHAPPEL, NEAR DRESDEN, GERMANY.

## EMULSIFIED SOLID GREASE.

No Drawing. Application filed April 8, 1925, Serial No. 21,698, and in Germany April 10, 1924.

The requirements in connection with the lubrication of the axles of trucks and tubs and consequently the demands made on the lubricants used for this purpose are totally different from those made on the lubrication and the lubricants for the axles of other types of vehicles. Hitherto lubricants capable of being extruded and consisting of machine greases thinned with oil have been used for lubricating the axles of such trucks. According to tests made, emulsified solid greases containing a far greater percentage of water than the solid greases used hitherto may be used for this purpose. Stiff greases known at present contain about five percent water as a maximum. The water content may amount to 50% and more. The best emulsifying agents for the mineral oils used for making the new solid greases are polymerized oils, such as "voltol" oil, with which or instead of which other oil-soluble emulsifying agents may be used, such as wool-fat, wool-fat alcohols, Montan wax and the like. Voltol oil is made in the following manner: Hydrocarbon oil is introduced into a vessel in which are a plurality of rotatable electrodes separated by a dielectric. The vessel is filled with hydrogen at a sub-atmospheric pressure. The electrodes are subjected to a potential ranging between 4300 and 4600 volts at 500 cycles per second, and a current intensity of 19 to 23 amperes. This current varies with the pressure in the apparatus. The oil in the chamber is caused to trickle over the electrode surfaces by the rotation thereof. The oil is kept at a temperature of between 60 and 80 degrees. The electrical discharges arising from the individual electrode plates convert the rotating electrodes which are covered with oil into a flame roll of rose violet color. The oil falling onto and trickling over the electrodes is subjected to the electrical oscillations previously mentioned. The oil, after it has been subjected to this type of electrical treatment, is then treated as below. The emulsification may for instance be effected by the atomized mineral oils, in which "voltol" oil or other oil-soluble emulsifying agents are dissolved, being brought together with the atomized water.

Voltol oil is introduced into an open boiler or container and heated by a current of steam until it no longer takes up any steam wherein at the same time the voltol oil is energetically agitated by the steam current passing from the oil. The water is then permitted to run into the voltol oil heated by the steam current, so that in all about 50 parts by weight of volume of water are added to the oil. If it is desired to produce very stiff grease we add to the voltol oil in the boiler paraffin wax, Montan wax or higher alcohols to the amount of 3-7% and with respect to the weight of the finished emulsion grease, according to the desired consistency.

The new emulsified solid greases with a high percentage of water completely fulfil as regards their properties all requirements as to the good lubrication of the axles of trucks. The moving parts subject to friction are moved on small spheres of water on the surface of the lubricating film. On the water evaporating, the lubrication will be pure oil lubrication without any detrimental effect due to friction, such as would occur if there were any soap present. The new solid greases having a high percentage of water have the further advantage of being cheap, in which respect they even surpass the tar oil extrudable greases, which have also been used hitherto.

The new emulsified solid grease can for instance be made from 50 parts of electrically treated oil of high viscosity (30-40° Engler at 100° C.) and 50 parts of water; or from 42 parts of thin liquid mineral oil, 6 parts of wax, 2 parts of highly viscous oil made by electric treatment and 50 parts of water; or from 42 parts of tar oils suitable for lubricating purposes, 6 parts of paraffin wax; 2 parts of highly viscous oil made by electric treatment and 50 parts of water.

What I claim is:—

1. An emulsified solid grease containing a relatively high percentage of water comprising mineral lubricating oil, water and

polymerized oil, said polymerized oil and lubricating oil being soluble in each other and said polymerized oil being in sufficient quantity to insure emulsification of said water in the lubricating oil.

2. An emulsified solid grease as defined in claim 1, containing in addition an oil soluble emulsifying agent comprising a higher alco-

hol, the amount of polymerized oil and higher alcohol being in sufficient quantity to ensure emulsification of the water in the lubricating oil. 10

In testimony whereof I have signed my name to this specification.

MORITZ JOSEPH HEITMANN.